

July 13, 1943.

J. F. FISCHER

2,324,377

PORCELAIN BUSHED GRINDING WHEEL

Filed July 23, 1942

FIG. 1.



FIG. 2.



FIG. 3.



FIG. 5.



FIG. 7.



FIG. 8.



Inventor:  
John F. Fischer  
by his Attorneys  
Kowar & Kowar

## UNITED STATES PATENT OFFICE

2,324,377

## PORCELAIN BUSHED GRINDING WHEEL

John F. Fischer, Drexel Hill, Pa., assignor to  
 Abrasive Company, Philadelphia, Pa., a corporation of Pennsylvania

Application July 23, 1942, Serial No. 452,041

5 Claims. (Cl. 51—206)

This invention relates to abrasive grinding implements, such as mounted wheels, mounted points, and various other types including wheels of different kinds, discs, cones, cups, cylinders, and segments. The invention relates particularly to abrasive grinding implements of the vitrified type, as distinguished from the resinoid and other non-vitreous types.

Commercial vitrified grinding implements are composed of a suitable granular abrasive substance, such as aluminum oxide, silicon carbide etc., bonded with a ceramic material having high vitrifying characteristics. The mixed bond and granular abrasive material is molded into appropriate shapes, which are subsequently subjected to a high vitrifying temperature, i. e. temperatures of approximately 2300° F., for effecting integration of the components, by fusing; while integration of the components of the implements of the resinoid type, for example, is effected at relatively low temperatures, i. e. temperatures approximating 360° F.

In the case of implements of smaller sizes, and particularly those of the vitrified type, each of the grinding implements is provided with a spindle or mandrel which is rigidly secured therein, and by which the grinding implement is mounted in the chuck of a stationary or portable grinding apparatus for operation. These spindles are usually knurled adjacent one end, and the knurled end is inserted and firmly cemented in a pre-formed axial cavity in the implement.

Under the present practice, the spindles are discarded, with the implements, when the implements are no longer usable.

The spindles are usually formed of high grade steel or steel alloy, which, in view of the present emergency, is extremely difficult to obtain, thus conservation thereof becomes of paramount importance.

In order to conserve the steel, the present invention is directed to the provision of vitrified abrasive grinding implements having interchangeable spindles, whereby a single spindle may be employed with an infinite number of different implements in succession.

It has been known in the art, heretofore, to provide abrasive wheels of the resinoid and other low temperature integrating types with interchangeable spindles. However, prior to the present invention, no satisfactory substitute for the integral spindle in the vitrified type of abrasive grinding wheel, point etc. has been evolved.

In the low temperature integrating types of implements, it has been known to place metal

bushings, with plain or threaded bores, in the molds in which the implements are shaped; and to mold the implements around the bushings before subjecting the molded articles to low firing temperatures required for effecting integration of the components thereof. This procedure is made possible by reason of the integrating temperature of the bonding material of the implement being lower than the fusing or scaling temperatures of the metal of which the bushings are composed.

It has also been known to provide threaded spindles for interchangeable mounting in the threaded bores of the metal bushings, in the low temperature integrating types of implements.

It has also been known to form axial cavities in other types of molded abrasive wheels and, thereafter, to fill such cavities with molten Babbitt metal, and to form plain bores in the metal plug during pouring thereof, or to drill and tap the plugs after solidification to receive threaded spindles.

Due to the extremely high integrating temperature of the vitrified implements, it is impractical to mold metal bushings therein, as the metal obviously would scale or fuse to such an extent as to render the bushings within the wheels etc. useless.

The filling of preformed cavities with babbitt metal for drilling and tapping to receive interchangeable spindles is unsatisfactory in most instances, due to the softness of the metal permitting the spindles to become loose in the wheels etc. in operation.

In accordance with the present invention, a satisfactory interchangeable spindle structure for vitrified abrasive grinding wheels etc. is made possible by the use of bushings which are composed of high grade ceramic material having a higher fusing temperature than the bonding material of the vitrified grinding implements. Preferably, these bushings are composed of a fine grain porcelain, as will be more fully disclosed hereinafter, reference being had to the accompanying drawing of which:

Fig. 1 is a longitudinal sectional view of a vitrified abrasive grinding implement in the form of a wheel or point provided with an internally threaded porcelain bushing and an interchangeable spindle, in accordance with the principles of the present invention;

Fig. 2 is a detached perspective view of the porcelain bushing shown in Fig. 1;

Fig. 3 is a longitudinal sectional view of the

vitrified abrasive grinding wheel of Fig. 1, in its "green" state, and the prefused bushing of Fig. 2 assembled prior to "firing," "burning" or "fusing" of the wheel;

Figs. 4, 5, 6, 7, and 8 illustrate modifications of the invention.

In accordance with the present invention, the porcelain bushings 3 of Fig. 2 are preferably composed of a fine grain porcelain of the steatite or similar type vitreous body of the better grade, such, for example, as are used in the manufacture of spark plugs for internal combustion engines etc.

The porcelain bushings 3, in accordance with the usual practice followed in the manufacture of spark plug porcelains and similarly high grade porcelainware, are preferably provided with a high gloss on the exterior surface thereof, which is produced by dipping or otherwise coating the articles, prior to final "firing" thereof, with a suitable glazing, after which porcelainware is usually fired at temperatures of approximately 2500° F.

A practical type of glazing substance which is adapted for use on the bushings 3, for the purpose of the present invention, is one which is generally known as an "empirical formula," as follows:



and of which the following batch weights are given as a practical example:

|                 | Parts by weight |
|-----------------|-----------------|
| Potash feldspar | 167             |
| Whiting         | 70              |
| Kaolin          | 52              |
| Flint           | 108             |

Glazing material of the foregoing type will fuse at temperatures approximating 2100° F.

In order to produce the implement shown in Fig. 1, for example, one of the prefired, externally glazed bushings 3, of Fig. 2, is secured in place in a mold having an interior configuration corresponding to the exterior shape of the body 1 of the wheel or point, after which the green unfired mixture of granular abrasive material and ceramic bond material, such as hereinbefore described, is compressed within the mold, around the insert 3, with the interior surface 2 of the compacted mixture in firm contact with the glazed exterior surface 4 of the insert 3.

After the "green" molded wheel 1 and prefired insert 3 are assembled, and removed from the mold as illustrated in Fig. 3, the assemblage is placed in a suitable oven or kiln and fired at temperatures of approximately 2300° F., as noted above. In the course of this firing, a fusion between the outer glaze 4 on the prefired porcelain insert 3 and the bonding agent forming and lying adjacent the surface 2 of that portion of the green wheel 1 immediately surrounding the insert 3 is effected, as indicated at 4a in Fig. 1. This fusion causes the porcelain bushing 3 to become an inseparable integral part of the wheel 1, whereby relative movement, either circularly or axially, between the bushing and the wheel is thereafter absolutely prevented.

During the course of manufacture of the porcelain bushings 3, each bushing is provided with an axial bore 5, which may be plain or provided with internal threads 6, as desired, the threads 6, under such circumstances, being formed during the molding of the bushings while the bushings are in their "green" prefired state.

As shown in Figs. 1 and 3, during the assembling of the finished bushings 3 and the green wheels 1 in the molds, the end surface 7 of the bushing 3 is aligned flush with the end surface 8 of the green wheel 1, and this relationship is maintained throughout the firing operation and until integration of the components of the wheel and simultaneous fusing thereof with the bushing 3 has been accomplished.

10 In accordance with the present invention, the threads 6 in the axial bore 5 of the bushing 3 are adapted to receive screw threads 9 which are formed on a spindle 10, along one end 11 thereof. The opposite end 12 of the spindle 10, in the present instance, is of plain circular form adapted for use in ordinary spindle-holding chucks. However, the outer ends 12 of the spindles 10 may be squared, tapered, or of any other desired cross-sectional or longitudinal shape without departing from the spirit of the invention.

Intermediate the threaded end 11 and the plain end 12 of the spindle 10, each spindle is provided with an annular flange or collar 13 which preferably is formed as an integral part of the spindle. The shoulder 14 of the flange 13 is adapted to abut firmly against the flat face 7 of the bushing 3.

It will be noted that the threaded end 11, of the spindle 10, beyond the face 14 of the flange 13, is shorter than the depth of the axial boring 5 of the bushing 3, whereby it would be impossible to thread the spindle into the boring 5 until the extreme end 15 of the spindle made contact with the base surface 16 of the bore 5, which, if subsequent relative rotation between the threaded spindle and the threaded bushing were effected, might cause the porcelain threads 6 to be stripped or broken by the metal threads on the end 11 of the steel spindle 10.

The jamming of the face 14 of the spindle flange against the face 7 of the bushing affords a rigid but readily detachable connection between the wheel and the interchangeable spindle 10.

45 While the inner ends of the bushings 3 have been shown as semispherical in Figs. 1, 2 and 3, and the body of the bushing has been shown as purely cylindrical, it will be understood that the inner ends of the inserts may be flat and open, as shown in Figs. 4 and 5, or flat and closed, as shown in Figs. 6, 7 and 8 or any other desired shape.

50 As illustrated in Figs. 4 and 5, the bushings 3c are open at both ends and provided in the axial bores thereof with screw threads 6c extending from end to end thereof or to a lesser extent if desired.

55 As illustrated in Figs. 6, 7 and 8, the closed ends 20, of the bushings 3a and 3b respectively, may be provided with transverse grooves, as indicated at 18 in Fig. 6, or transverse ribs as indicated at 19 in Figs. 7 and 8, while the bodies of the bushings may be cylindrical, rectangular or polygonal, if desired, without departing from the spirit of the invention, deviation from the cylindrical form or the spherical inner end being provided, in some instances if desired, to assure against relative circular movement between the prefired bushing and the "green" body of the wheel while being removed from the molds and while being placed in the kiln. Such relative movement may impair the otherwise snug fit between the outer glazed surface 4 of the bushing 3 and the surface 2 of the green material of the implement before fusion 75 therebetween is effected.

The bushings 3a, 3b and 3c of Figs. 5, 6, 7 and 8 are adaptable for use in the wheel or point type of implement, as shown in Fig. 1, to receive the threaded end of the interchangeable spindle 10, or these bushings may also be used in the disc type of vitrified implement 1c, shown in Fig. 4, for securing a backing plate 25 to the disc, in which case a series of the inserts 3c are placed in and integrated with the body 1c of the disc at a number of relatively spaced points, about the axis of the disc, to receive the threaded ends 11c of suitable bolts 10c by which the backing plate 25 of metal or other suitable material is secured to one side of the grinding disc.

It will be understood that the inserts of the present invention are preferably of ordinary composition as employed in the manufacture of porcelainware of the commercial varieties of the better grades, i. e. those using a fine grain base, such as talc, and any of the usual commercially employed glazings, which are susceptible to fusion with the vitreous bonding agent of the abrasive grinding implements. The composition of the implements likewise is preferably the same as commercially used in the art, no special ingredient being required in either the composition of the implements, the composition of the insert, or the composition of the glaze employed on the bushing in order to practice the present invention successfully.

I claim:

1. A vitrified abrasive grinding implement, and a prefired ceramic insert embedded therein prior

to firing of said implement and fused therewith by subsequent firing of said implement.

2. A vitrified abrasive grinding implement formed of granular abrasive material and a bonding material of relatively high fusing temperature, a prefired ceramic insert having a relatively higher fusing temperature embedded in said implement and an intermediate fluxing substance having a fusing temperature less than said bonding material for uniting said insert and said implement.

3. A vitrified abrasive grinding implement formed of granular abrasive material bonded with a bonding material of relatively high fusing temperature, a ceramic insert including a bonding material of relatively higher fusing temperature embedded in said implement, and a glazing material on the embedded surfaces of said insert and fusible at a temperature consistent with the fusing temperature of the bond of said implement for fusing said insert with said implement as an inseparable integral part thereof.

4. A vitrified abrasive grinding implement and a prefired porcelain bushing embedded therein prior to firing of said implement and fused therewith by subsequent firing of said implement.

5. A vitrified abrasive grinding implement and a prefused externally glazed porcelain bushing embedded therein prior to firing of said implement and fused therewith through said glaze by subsequent firing of said implement.

JOHN F. FISCHER.